

## UNITED STATES PATENT OFFICE

2,304,659

## STEREOTYPE MAT

Arlie W. Schorger, Madison, Wis., assignor to  
Burgess Cellulose Company, Freeport, Ill., a corporation of Delaware

No Drawing. Application October 17, 1940,  
Serial No. 361,606

11 Claims. (Cl. 22--5.5)

This invention relates to stereotype mats, particularly those known as dry mats, and is directed to the improvement of such mats whereby their molding and casting properties are improved. The invention relates to the improved stereotype mat and to the method of making the same.

It is the object of the invention to provide a stereotype mat having improved plasticity during molding whereby it is adapted to receive a deep, sharp, and clear-cut impression from the mold with a minimum of fracture in the face.

It is also an object of the invention to provide an improved stereotype mat which will give a large number of casts which are excellent reproductions of the pattern.

The stereotype mat which is in common use is a relatively thick, moisture-absorbent fibrous sheet which is composed of cellulose fibers, such as rag stock, cotton linters and chemical wood pulp, usually sulfite pulp. It usually contains a filler, such as clay, talc, etc., mixed with the fibers. Examples of such stereotype mats are disclosed in my United States Patents 1,524,155, granted January 27, 1925, and 1,720,243, granted July 9, 1929. The surface of the mat which is to receive the impression of the mold may be given a coating to improve its uniformity and smoothness. An example of such a coating treatment is disclosed in my Patent 1,863,731, granted June 21, 1932.

The mat is moistened for the operation of receiving the impression from the pattern, and in this condition must be capable of readily undergoing compression and stretch in order to form an exact reproduction of the pattern which often contains fine details. After the molding operation, the mat is dried, and in this condition it must be hard and have a uniformly smooth surface in order that a large number of accurate reproductions may be made by casting molten stereotype metal against it. If fractures are present, the molten metal flows into them, and removal of the solidified metal causes tearing of the surface of the mat. The present invention results in improved plasticity for the molding operation, and improved smoothness and freedom from fracture for the casting operation.

Plasticity of the mat in its moistened condition is of utmost importance in order that the mat may take, readily, and without the application of excessive pressure, a full and exact impression of the pattern or form. Cellulose fibers themselves, possess only limited plasticity, the impression taken by the mat being due largely to the compression and stretch which the fibers undergo. A sheet of cellulose fibers has characteristic limitations with respect to compression and stretch, and it is the purpose of the present

invention to provide a stereotype mat in which these properties are modified to advantage.

In accordance with the present invention, it has been discovered that if certain proteins, in finely divided condition, are incorporated among the fibers of the stereotype mat, the plasticity of the mat when moistened is greatly increased. A stereotype mat is usually made upon a paper making machine, and the mat of this invention may be made in the same way. The finely divided protein and cellulose fibers are intimately mixed and suspended in water and are then formed into a sheet of the desired thickness. The sheet is then dried and calendered to produce the desired smooth-surfaced stereotype mat. A filler such as is usually used in the stereotype mat art, for example, clay, talc, etc., may be mixed with the fibers and protein and thus incorporated in the resulting mat.

Suitable proteins are the vegetable proteins and casein. Casein is derived from milk and is commonly considered to be an animal protein. In reality it is closely related to vegetable proteins and is not so far removed from the vegetable protein from which it is derived that it has lost the essential characteristics of vegetable protein.

Many vegetable products which are high in protein may be used. While the protein may be isolated from the natural vegetable product for use in the invention, it is satisfactory, and usually more economical, to use the protein-bearing vegetable products in their natural state, and merely comminute them to the desired particle size. Some of the commercially obtainable protein-bearing vegetable products which may be used are given in the following list, the approximate content of protein therein being given opposite each item. The percentages are of protein in the crude form, since it does not need to be refined for the purposes of this invention.

|                                                             | Crude protein per cent |
|-------------------------------------------------------------|------------------------|
| Cottonseed meal                                             | 33-44                  |
| Hemp cake                                                   | 31                     |
| Linseed meal                                                | 33-43                  |
| Brewer's grains                                             | 18-28                  |
| Peanut meal                                                 | 38-48                  |
| Velvet beans                                                | 26                     |
| Pea                                                         | 25                     |
| Navy bean                                                   | 23                     |
| Corn gluten meal                                            | 43                     |
| Corn germ meal                                              | 21                     |
| Corn protein product marketed under the trade mark "Mazein" | 100                    |
| Soybean meal                                                | 38-48                  |

Some of the vegetable products, such as cottonseed meal and linseed meal, contain a relatively large proportion of oils and fats. In such case, it is preferable that most of the oil and fat

be removed by expression or extraction before the material is incorporated in the mat.

The quantity of protein which may be incorporated in the stereotype mat may vary over a considerable range. As little as 5% of protein, based upon the dry weight of the stereotype mat, produces a pronounced effect in increasing the plasticity. The effect is augmented with increasing protein content, and a 50% protein content provides plasticity of a very high order. This is the maximum protein content which it is desirable to employ. The preferred range is from 10% to 30% of protein. Where a natural protein-bearing material is employed, and the mat contains a filler, the mat is composed of cellulose, filler, protein and the non-protein constituents of the protein-bearing material. The cellulose fibers impart firmness and strength to the mat, and it is desirable that the cellulose content of the stereotype mat be at least 20% of the total solids. As an example of the present invention, a stereotype mat is made of a mixture which is 60% by weight of cellulose fibers and 40% by weight of soybean flour. Such a stereotype mat contains approximately 16% of crude protein.

The molding operation is carried out at room temperature or at an elevated temperature, depending upon the practice of the particular user. The increase of plasticity is realized in either case. The air-dry moisture content of the stereotype mat is from 5% to 8%, and prior to the molding operation, it is moistened until it has a water content of approximately 10% to 50%, based upon the weight of the mat. In this condition, it is pressed against the form which carries the printing or other characters or design which it is desired to reproduce. This form may be either hot or cold, as explained heretofore. In either case, the mat containing protein possesses greater plasticity to a pronounced degree in comparison with a similar mat which does not contain protein. The plasticity is somewhat higher if a hot form is used. As a result, a deep mold is obtained with moderate pressure, and fine details are reproduced with great accuracy. After the molding operation, the stereotype mat is dried by means of suitable drying apparatus. For this operation, it may be removed from the form, or the form, without disturbing the mat, may be transferred to the drying apparatus. After the mat is dry, it has a uniformly smooth hard surface, free of fractures, and many casts can be made from it.

The mat of this invention provides the additional advantage that it possesses greatly increased plasticity even when the moisture content is low. A moisture content of from 10% to 15% is sufficient to realize the advantage of high plasticity. The time and cost of drying is reduced as a result. Savings in time are of essential importance where the mat is being used in a newspaper plant.

Suitable antiseptics for preventing or retarding the growth of molds and bacteria are incorporated in the mat.

In the foregoing description, the protein is in a finely divided solid condition when it is incorporated with the cellulose fibers. It may be incorporated in the dissolved condition, also. For this purpose, the protein is brought into solution in a suitable aqueous alkaline solution, for example, a solution of a carbonate or hydroxide of an alkali metal. This solution is then mixed with the cellulose fibers, and the mass is

treated with an acid to neutralize the alkali and precipitate the protein in situ. For convenience and simplicity and also for the most satisfactory results, it is preferred that the protein be in the finely ground solid state. The particles should be sufficiently fine that substantially all pass through a 100 mesh per inch sieve (particle diameter 0.0059 inch), and preferably through a 200 mesh per inch sieve (particle diameter 0.0029 inch).

The protein may be treated with an aldehyde, such as formaldehyde, or with an tannin, and the plasticity obtained by the use of such treated protein in the stereotype mat is substantially the same as that obtained when protein itself is used.

The following are several specific examples of methods for carrying out the present invention. It is understood that the invention is not limited to these specific methods, but only in accordance with the scope of the appended claims.

#### Example No. 1

A water suspension is made containing 60 parts by weight of cellulose fibers, 40 parts of soybean flour which has been ground to a size which will pass through a 200 mesh per inch sieve, and 50 parts of clay. The whole is mixed uniformly and then the solids are felted into a sheet of the desired thickness on a paper machine in a manner well known to those skilled in the art, and the sheet is dried and calendered. The thickness of the finished sheet may vary from 0.015" to 0.036", as desired. The dried and calendered sheet is then humidified until it has taken up moisture sufficient to produce a water content of from 10% to 50%, depending upon the moisture requirements for the particular application. After the moisture becomes distributed uniformly, the sheet is ready for the molding operation.

#### Example No. 2

A water suspension containing 80 parts of cellulose fibers, 50 parts of clay, and 20 parts of casein, ground to pass through a 200 mesh per inch sieve, is mixed thoroughly. A mat is formed from this suspension in a manner similar to that described in Example 1.

Satisfactory results are obtained employing similar quantities of "Mazein" in place of casein in the procedure of this example.

#### Example No. 3

A water suspension is made of an intimate mixture of 100 parts of cellulose fibers, 40 parts of cottonseed flour (approximately 15 parts of crude protein) and 5 parts of talc. The procedure of forming the stereotype mat from the suspension is the same as in Example 1.

#### Example No. 4

A water suspension is made composed of a mixture of 100 parts of cellulose fibers, 40 parts of linseed flour (approximately 10 parts of crude protein) and 50 parts of talc, the subsequent procedure being similar to that of Example 1.

Excellent results are obtained if 40 parts of pea flour (approximately 10 parts of crude protein) is employed in the procedure of this example in place of the linseed flour.

The term "protein" as employed in the claims is intended to cover the natural protein-bearing vegetable substance as well as the isolated protein, and where proportions are given, they repre-

set proportions of the isolated protein. While it is stated throughout the specification that the protein is in crude form, the invention is not limited to such protein, and refined protein may be used as well.

I claim:

1. A fibrous stereotype mat having incorporated among and in intimate mixture with the fibers thereof, at least approximately 5%, based on the weight of said stereotype mat, of finely divided particles of protein from the group consisting of vegetable protein and casein.

2. A fibrous stereotype mat having incorporated among and in intimate mixture with the fibers thereof, finely divided particles of an inorganic filler and of protein from the group consisting of vegetable protein and casein, said protein and fibers comprising, respectively, at least approximately 5% and 20% of the weight of said mat.

3. A fibrous stereotype mat having incorporated among and in intimate mixture with the fibers thereof, at least approximately 5%, based on the weight of said stereotype mat, of finely divided particles of protein from the group consisting of vegetable protein and casein, substantially all of said particles being of a size adapted to pass through a 100 mesh per inch sieve.

4. A fibrous stereotype mat having incorporated among and in intimate mixture with the fibers thereof, at least approximately 5%, based on the weight of said stereotype mat, of finely divided particles of protein from the group consisting of vegetable protein and casein, substantially all of said particles being of a size adapted to pass through a 200 mesh per inch sieve.

5. A fibrous stereotype mat having incorporated among and in intimate mixture with the fibers thereof from approximately 5% to approximately 50%, based on the weight of said stereotype mat, of finely divided particles of protein

from the group consisting of vegetable protein and casein.

6. A fibrous stereotype mat moistened with water and having incorporated among and in intimate mixture with the fibers thereof, at least 5% based on the dry weight of said stereotype mat, of finely divided particles of protein from the group consisting of vegetable protein and casein.

7. A fibrous stereotype mat having a water content of from 10% to 50% of the total weight thereof, and having incorporated among and in intimate mixture with the fibers thereof, at least approximately 5%, based on the dry weight of said stereotype mat, of finely divided particles of protein from the group consisting of vegetable protein and casein.

8. A sheet-form fibrous stereotype mat having a thickness of approximately 0.015" to 0.036", said mat being composed of cellulose fibers and having incorporated among and in intimate mixture with the fibers thereof, at least approximately 5%, based on the weight of said stereotype mat, of finely divided particles of protein from the group consisting of vegetable protein and casein.

9. A fibrous stereotype mat having soy bean flour distributed among and in intimate mixture with the fibers thereof, the protein of said soy bean flour comprising at least approximately 5% and the fibers at least approximately 20%, of the weight of said stereotype mat.

10. A fibrous stereotype mat having incorporated among and in intimate mixture with the fibers thereof, at least approximately 5%, based on the weight of said stereotype mat, of finely divided particles of vegetable protein.

11. A fibrous stereotype mat having incorporated among and in intimate mixture with the fibers thereof, at least 5%, based on the weight of said stereotype mat, of finely divided particles of casein.

ARLIE W. SCHORGER.